

## UNITED STATES PATENT OFFICE.

FERNANDO SOMOZA VIVAS, OF LOS ANGELES, CALIFORNIA.

## FIREPROOF VARNISH.

No Drawing. Application filed June 14, 1923, Serial No. 645,344. Renewed May 26, 1926.

The invention relates to fire-proof varnish, and has as an object the provision of a material of this character which is non-inflammable, and which when applied to inflammable materials will prevent them from being burned. A further object of the invention is the provision of a fire-proof varnish that will be weather resistant so as to be efficient for the usual function of a varnish, namely to prevent deterioration of the surfaces to which it is applied by weathering or the wear of use. A further object of the invention is the provision of a fire-proof varnish which will be comparatively cheap to produce.

The formula for the varnish embodying the invention which it is preferred to use with the proportions of the different ingredients is as follows:

|                            | Parts. |
|----------------------------|--------|
| Drying oil                 | 45     |
| Varnish gum                | 50     |
| Glycerine                  | 5      |
| Lime                       | 1      |
| Cobalt acetate             | 1      |
| Lead acetate               | 1      |
| Thinner                    | 10     |
| Borax                      | 15     |
| Boric acid                 | 8      |
| Tungstate of sodium        | 3      |
| Perchlorethane ( $CCl_3$ ) | 2      |

The thinner above listed, in the above formula, is made the subject-matter of a co-pending application filed June 14, 1923, Serial Number 645,346 and the formula of the same is as follows:

|                      | Parts. |
|----------------------|--------|
| "Nearturps"          | 40     |
| Turpentine           | 10     |
| Zinc sulphate        | 5      |
| Perchlorethane       | 1      |
| Drying oil           | 4      |
| Carbon tetrachloride | 40     |

The "Nearturps" in the above solvent formula is a mineral oil product which is in common use to replace some of the turpentine in the mixture of paints. The substance is a gasoline produced by straight distillation, as distinguished from a cracking process, and which has been deodorized by treatment with alcohol. Other turpentine substitutes may be used in lieu thereof if desired.

The oil in either formula may be linseed oil or any accepted equivalent thereof, and the varnish gum may be any of the usual gums from which varnishes are made. While both cobalt acetate and lead acetate have been recited in the formula, one or the other thereof may be omitted without destroying the fireproof or other qualities of the varnish.

Minor changes may be made in the proportions of the parts, or known equivalents may be utilized for any of the ingredients named without departing from the spirit of the invention.

## I claim:

1. A varnish comprising in combination, drying oil, varnish gum, glycerine, lime, an acetate, a thinner, borax, boric acid, tungstate of sodium and perchlorethane, in proportions to form a fireproof varnish.

2. A fire-proof varnish comprising in combination, drying oil 45 parts, varnish gum 50 parts, glycerine 5 parts, lime 1 part, cobalt acetate 1 part, lead acetate 1 part, a thinner 10 parts, borax 15 parts, boric acid 8 parts, tungstate of sodium 3 parts and perchlorethane 2 parts.

3. A fire-proof varnish comprising in combination, drying oil, varnish gum, glycerine, lime, cobalt acetate, lead acetate, borax, boric acid, tungstate of sodium, perchlorethane, "Nearturps," turpentine, zinc sulphate, and carbon tetrachloride in proportions to form a fire-proof varnish.

FERNANDO SOMOZA VIVAS.